# EUROPEAN PATENT SPECIFICATION

(11) **EP 0 190 114 B1**
(45) Date of publication and mention of the grant of the patent: **05.04.1989**
(21) Application number: 86850031.5
(22) Date of filing: 31.01.1986
(51) Int. Cl.: B22D 19/00

(54) **Molded metal object and method to manufacture the same**
Metallgussstück und Verfahren zu seiner Herstellung
Pièce coulée en métal et son procédé de fabrication

(30) Priority: 01.02.1985 SE 8500474
(43) Date of publication of application: 06.08.1986
(73) Proprietor: AB VOLVO, 405 08 Göteborg (SE)
(72) Inventor: Lindgren, Hâkan, S-73400 Hallstahammar (SE); Björklund, Nils-Eric, S-73400 Hallstahammar (SE); Carlsson, Jan-Olov, S-54141 Skövde (SE)
(74) Representative: Säfwenberg, Björn

(56) References cited:
- EP-A- 0 071 047
- DE-B- 1 285 680
- FR-A- 2 431 335
- PATENTS ABSTRACTS OF JAPAN, vol. 8, no. 67 (C-216) [1504], 29th March 1984; & JP - A - 58 217 671 (MITSUBISHI JUKOGYO K.K.) 17-12-1983

## Description

The invention relates to a method to manufacture a molded metal object of the kind stated in the preamble of claim 1. The invention also relates to a molded metal object manufactured by such a method.

The background of the invention is a desire to achieve a molded metal object comprising one or more channels or cavities, the internal surfaces of which are formed by sprayed layers of a high temperature and corrosion resistant metal alloy.

According to one previously known method, prefabricated, thermally sprayed tubes can be molded into an object with a remaining mandrel or core. Then it has only been possible to use tubes with a simple, especially cylindrical shape, since the mandrel or core must be removed after molding.

According to a second known method (EP-A-0 071 047), corresponding to the preamble of claim 1, a prefabricated tube or shell is mounted in a mold, whereupon the tube or shell is filled with sand and the object is molded around the tube or shell. However, in this known method, the molding is performed without removing the original core, resulting in a deterioration in the bonding material of the sand core and difficulty in retaining the tube or shell in exact position in the mold. In fact, the function of the sand is only to retain the shape of the tube or shell during the molding process. ^{t}

Other known methods of molding are disclosed in FR-A-2431 335 and DE-B-1 285 680, wherein a channel or cavity for a combustion engine is formed by flame spraying a metal alloy onto a sand core, which is then placed in a sand mold, whereupon a metal material is molded around the tube or shell previously formed. However, the tube or shell is not refilled with sand before the molding process.

The object of the invention is therefore to provide a method to manufacture a molded metal object having at least one internal channel or cavity of a complicated configuration, and this object is achieved by the steps of
producing said tube or shell by thermal spraying of a high temperature and corrosion resistant metal alloy onto a core body,
removing said core body so as to leave a self-supporting tube or shell,
making a sand mold for the object to be molded, said self-supporting tube or shell being mounted into a tool for making the sand mold and being refilled with molding sand, and
molding said object in said sand mold around the refilled tube or shell.

Hereby, it is possible, practically without any restrictions, to provide any desired configuration of the cavities or channels of the metal object. It is important that the core body is removed during or after the prefabrication of the tube or shell and that the tube or shell is refilled with molding sand when making the sand mold.

By removing the original sand core body, it is possible to spray two or more additional layers onto the first metal alloy layer (cf. claim 2), while permitting the first layer to expand and shrink freely. The subsequent refilling of the self-supporting tube or shell ensures that the latter is retained in exact position during the molding process.

The invention also concerns a molded metal object manufactured by the method indicated above, as defined in claims 3 and 4.

The invention will be explained further below with reference to the appended drawings schematically illustrating an embodiment in which the tube is made by thermal spraying onto a sand core.
Fig. 1 shows a sand core onto which a metal alloy is to be thermally sprayed ;
Fig. 2 shows the sand core having a sprayed, thin first layer ;
Fig. 3 shows the tube to be molded into an object after removal of the sand core and spraying a relatively thick second layer onto the first layer ;
Fig. 4 shows schematically a molded metal object with a tube molded therein so as to form a channel in the metal object.

In a way known per se, a core body 1 is made of molding sand containing phenol resin as a binding agent. As shown in Fig. 1, this core body 1 has an external configuration corresponding to the desired, internal configuration of the tubular object, and additionally holding portions 1a, 1b at each end for holding the core body. In the embodiment, the desired object consists of an exhaust channel in a cylinder head in a combustion engine.

In accordance with Fig. 2, a relatively thin and essentially pore-free layer 2 of a metal alloy containing about 5 % Al, 22 % Cr and the rest mainly Fe (the contents are by weight) is sprayed onto the core body. When the layer thickness amounts to at least 0.5 mm, preferably about 1 mm, the spraying operation is interrupted, whereupon the sand core 1 is removed by heating the sprayed sand core in a furnace at about 600 °C during 2-3 hours, and thereafter discharging the sand from the thin, tubular metal alloy layer 2.

Thereafter, a second layer 3 is sprayed externally onto the first, self-supporting thin layer 2. In absence of a core body, the first layer 2 is permitted to expand and shrink freely due to variations of temperature, without any risk of tensions and accompanying cracking. The thickness of the second layer may be at least 1.5 mm. The spraying process can be performed without interruption for cooling.

Different methods of spraying are possible. Preferably, the first, relatively thin layer 2 is sprayed by means of a wire-fed flame sprayer so as to form a dense layer. In case a surface layer with great purity is desired (small quantities of oxides and pores), the layer may be applied by plasma spraying. The second layer 3 may preferably be applied by means of a powder-fed flame sprayer in order to obtain a suitable quantity of pores and oxides. In this case a total quantity of 5-25 %, preferably about 15 %, pores and oxides is desired.

However, the second layer 3 does not have to be of the same material composition as the first layer 2, but may consist of another metal alloy with high heat resistance or of a ceramic material. However, there are no requirements of corrosion resistance.

Thereupon, the prefabricated tube 2,3 is mounted into a tool for the manufacture of a sand mould for the desired metal object. The tube 2,3 is again filled with sand, in order to enclose the corresponding part of the sand mould. Thereafter, the metal object is molded in a conventional way, wherein the tube 2,3 forms a channel, as schematically shown in Fig. 4. (In practice, the external outline of the metal object has a complicated geometry but is shown, for the sake of simplicity, as a box-like object).

Thus, the channel formed by the tube 2,3 molded therein has an internal surface consisting of the first sprayed layer 2, which is esentially pore-free and resistant against high temperatures and corrosive gases. Therefore, this layer may serve as an exhaust channel in a combustion engine. On the other hand, the second layer 3 being located inside the surface layer 2 has more pores and oxides and is also thicker, and it will therefore serve as an effective heat barrier against the other material in the metal object.

Naturally, by the method according to the invention, one may make metal objects of practically any configuration of internal cavities and channels by prefabricating shell or tube bodies of a corresponding geometry. Cavities may also form a part of the outside of the metal object, i. e. in order to form, together with another object, a space exposed to intense heat and corrosive gases, e. g. a combustion chamber, a valve chamber, an exhaust channel or the like.

The tube or shell to be molded into the metal object can be produced by methods other than thermal spraying, such as e. g. a powder metallurgical process or plate pressing. It is also possible to press a thin plate into a tube or shell and therafter apply at least one layer of a heat and corrosion resistant metal alloy by thermal spraying.

Compared with prior art technology, the following advantages are obtained :
complicated cavities or channels may be prefabricated quickly and simply and thereafter molded into a metal object ;
the handling becomes easier and the waste will be less ;
the molding precision is increased ;
compared with applying ceramic material as a surface layer, the inventive method is cheaper and better due to good metal-to-metal adherence, and there are no problems with expansion due to varying temperatures.

## Claims

1. A method to manufacture a molded metal object having at least one channel and/or cavity, especially intended to be incorporated in a combustion engine, wherein a tube or a shell, the internal dimensions of which correspond to said channel or cavity, is prefabricated, whereupon the prefabricated tube or shell is filled with sand and the object is molded around the tube or shell, characterized by the steps of
- producing said tube or shell by thermal spraying of a high temperature and corrosion resistant metal alloy onto a core body,
- removing said core body so as to leave a self-supporting tube or shell,
- making a sand mold for the object to be molded, said self-supporting tube or shell being mounted into a tool for making the sand mold and being refilled with molding sand, and
- molding said object in said sand mold around the refilled tube or shell.

2. A method as defined in claim 1, characterized in that a second, relatively thick second layer is thermally sprayed onto said layer upon removing said core body.

3. A molded metal object manufactured by the method defined in claim 1, characterized in that said tube (2,3) or shell comprises, on the one hand, a first, relatively thin and essentially pore-free layer (2) forming a wall surface in said channel or cavity, respectively, and, on the other hand, a second, relatively thick layer (3).

4. A molded metal object manufactured by the method defined in claim 1 or 2, characterized in that said tube (2,3) or shell comprises a layer consisting of 1-12 % AI, 10-30 % Cr, possibly small quantities of one or more elements in the group Si, Mn, Co, Y, Hf, possibly small quantities of oxides and nitrides, and the rest Fe.

## Patentansprüche

1. Ein Verfahren zur Herstellung eines geformten Metallgegenstandes mit wenigstens einem Kanal und/oder Hohlraum, insbesondere zum Einbau in einen Verbrennungsmotor, wobei ein Rohr oder eine Hülse, deren Innenabmessungen dem Kanal oder Hohlraum entsprechen, vorgefertigt wird, worauf das vorgefertigte Rohr oder die vorgefertigte Hülse mit Sand gefüllt und der Gegenstand um das Rohr oder die Hülse herum geformt werden, gekennzeichnet durch die Schritte :
- Herstellen des Rohres oder der Hülse durch thermisches Aufsprühen einer hochtemperatur-und korrosionsbeständigen Metallegierung auf einen Kernkörper,
- Entfernen des Kernkörpers, so daß ein selbsttragendes Rohr oder eine selbsttragende Hülse verbleibt,
- Herstellung einer Sandform für den zu formenden Gegenstand, wobei das selbsttragende Rohr oder die selbsttragende Hülse in ein Werkzeug für die Herstellung der Sandform eingesetzt und wieder mit Formsand gefüllt wird, und
- Formen des Gegenstandes in der Sandform um das wiedergefüllte Rohr oder die wiedergefüllte Hülse herum.

2. Ein Verfahren nach Anspruch 1, dadurch gekennzeichnet, daß eine zweite, relativ dicke Schicht nach Entfernung des Kernkörpers auf besagte Schicht thermisch aufgesprüht wird.

3. Ein geformter Metallgegenstand, hergestellt durch das Verfahren nach Anspruch 1, dadurch gekennzeichnet, daß das Rohr (2,3) oder die Hülse einerseits eine erste, relativ dünne und im wesentlichen porenfreie Schicht (2) umfaßt, die eine Wandfläche in dem Kanal bzw. Hohlraum bildet, und andererseits eine zweite, relativ dicke Schicht (3).

4. Ein geformter Metallgegenstand, hergestellt durch das Verfahren nach Anspruch 1 oder 2, dadurch gekennzeichnet, daß das Rohr (2,3) oder die Hülse eine Schicht umfaßt, die aus 1 % bis 12 % Al, 10 % bis 30 % Cr, gegebenenfalls kleinen Mengen an einem oder mehreren Elementen der Gruppe Si, Mn, Co, Y, Hf, gegebenenfalls kleinen Mengen an Oxiden und Nitriden und im übrigen aus Fe besteht.

## Revendications

1. Procédé de fabrication d'un objet métallique moulé présentant au moins un canal et/ou une cavité, destiné notamment à être incorporé à un moteur à combustion, dans lequel on remplit de sable un tube ou une coque à dimensions internes correspondant audit canal ou à ladite cavité et l'on moule l'objet autour du tube ou de la coque, caractérisé par les opérations consistant à :
- fabriquer ledit tube ou ladite coque par projection à chaud d'un alliage métallique résistant aux hautes températures et à la corrosion sur un corps de noyau,
- extraire ledit corps de noyau afin de laisser un tube ou une coque autoportant,
- fabriquer un moule en sable de moulage de l'objet a mouler, ledit tube ou ladite coque autoportant étant monté à l'intérieur d'un outil de fabrication du moule en sable et étant rempli à nouveau de sable de moulage, et
- mouler ledit objet dans ledit moule en sable autour du tube ou de la coque rempli à nouveau.

2. Procédé selon la revendication 1, caractérisé en ce qu'on projette à chaud une seconde couche, relativement épaisse, sur ladite couche après avoir retiré ledit corps de noyau.

3. Objet métallique moulé fabriqué par le procédé selon la revendication 1, caractérisé en ce que ledit tube (2,3) ou ladite coque est constitué, d'une part, par une couche relativement mince et sensiblement exempte de pores (2) formant une surface de paroi dans ledit canal ou ladite cavité et, d'autre part, par une seconde couche relativement épaisse (3).

4. Objet métallique moulé fabriqué par le procédé selon la revendication 1 ou 2, caractérisé en ce que ledit tube (2,3) ou ladite coque comprend une couche composée de 1 à 12 % d'AI, de 10 à 30 % de Cr, éventuellement de faibles quantités d'un ou plusieurs éléments du groupe Si, Mn, Co, Y, Hf, éventuellement de faibles quantités d'oxydes et de nitrures, et pour le reste de Fe.
